

(No Model.)

2 Sheets—Sheet 1.

H. H. EAMES.  
METHOD OF TREATING ORES.

No. 529,441.

Patented Nov. 20, 1894.



## Witnesses

Anelia Williams.

Henry Shattock

Fig. 1.

## Inventor

Henry. H. Earnes.

(No Model.)

2 Sheets—Sheet 2.

H. H. EAMES.  
METHOD OF TREATING ORES.

No. 529,441.

Patented Nov. 20, 1894.



Fig. 3.



Fig. 4.



Fig. 5.

Witnesses

Audia Williams.

Henry B. Lathe.

Inventor

Henry H. Eames.

# UNITED STATES PATENT OFFICE.

HENRY H. EAMES, OF DETROIT, MICHIGAN, ASSIGNOR TO JOHN M. NICOL,  
TRUSTEE, OF SAME PLACE.

## METHOD OF TREATING ORES.

SPECIFICATION forming part of Letters Patent No. 529,441, dated November 20, 1894.

Application filed October 9, 1893. Serial No. 487,682. (No specimens.)

To all whom it may concern:

Be it known that I, HENRY H. EAMES, of Detroit, in the county of Wayne and State of Michigan, have invented a new and useful 5 Improvement in Methods of Treating Ores, of which the following is a specification.

My invention consists in an improved method of the treatment of ores, known as sulphides, arsenides, tellurides, and others of 10 the same class, in which the sulphur, arsenic, tellurium, or like substance, is separable from the ore by sublimation or distillation.

The object to be attained is, first, the separation from the ore of substances such as arsenic, tellurium, zinc, antimony, and the like, which are separable by distillation or sublimation, and the securing of these substances in marketable condition in the form of arsenic, sulphurous acid, arsenious acid, white 15 oxide of zinc, and the like, according to the process employed; second, the alteration of the structure and composition of ores containing precious metals, so that these metals may be reclaimed in metallic form by any of the 20 known methods.

The drawings illustrate an apparatus which may be used to practice my process, in which—

Figure 1 is a vertical central section. Fig. 2 is a section on line  $x-x$ , Fig. 1. Fig. 3 is a 25 partial elevation, partly in section, and Figs. 4 and 5 are a side view and plan view of a slightly modified form of grate.

A represents a furnace, of any suitable construction provided with a fire chamber A' having a grate B, and fire and ash pit doors 30 L and M.

G represents a chamber contained within the furnace A, an annular space D being left between the outside of chamber G and the in- 35 side of furnace A.

C represents a flue which connects the combustion chamber of A' with space D.

N N represent baffle plates alternately closing opposite sides of space D to force the 40 products of combustion to travel around chamber G, and H represents a smoke flue.

K represents a grate which closes the bottom of chamber G, and this grate is preferably made in two halves, as shown, hinged to 45 the bottom of the chamber, and provided with controllable air openings, Figs. 4 and 5 illus-

trating them made like registers, with one fixed and rotary point, provided with slots.

J is a pit under chamber G into which the contents of said chamber can be dumped. 55

I P is an exhaust pipe leading from the top of chamber G to one or more condensers of any known type, and I prefer to hinge the elbow I to the main pipe P at F, for convenience in charging.

E E represent air channels, or tuyeres, opening into chamber G at various levels by which air can be admitted to the chamber at will. Tuyeres E E are provided with valves O, (illustrated as of the register type,) by 65 which air can be admitted into the chamber at different zones and in regulated quantity.

For the treatment of ores containing gold and silver, zinc or arsenic, tellurium or antimony, the operation is as follows; an ore containing zinc being chosen for description: By means of a fire in furnace A, the chamber G is first heated to the proper temperature, (about a bright red,) and then is charged with broken ore. The top of chamber G is then 70 connected to the condenser by elbow I. All the air openings into the chamber G are closed, and the fire is maintained in the furnace until the ore is sufficiently heated to volatilize the zinc. When this heat is attained, 75

the air openings at the bottom and lower air openings at the sides of the chamber G are partly opened, and sufficient air is permitted to enter the chamber to oxidize the zinc. The progress of the operation may be ascertained 80 by inserting a rod through the different air openings E. The rod will be more or less coated with oxide of zinc. The upper part of chamber G above the charge acts as a combustion chamber, to thoroughly oxidize at 85 this point any zinc which may have reached that part of the chamber without being previously oxidized. When the lower portion of the charge has been depleted of the zinc 90 therein contained, the bottom air ports are fully opened and the air ports next above are partly opened, thus oxidizing the zinc contained in the ore in the second zone of the chamber G, the process being aided by the air which enters through the bottom and 95 lower air ports, and which becomes highly heated by passing up through the mass of in-

60

70

75

80

85

90

95

100

candescent material. In this manner I proceed upward from zone to zone, and the operation is complete when a rod inserted through the highest air openings does not collect any white oxide of zinc. The chamber G is then discharged by opening the hinged bottom K, the elbow I being first disconnected. Any precious metals which the ore may contain, as well as any base metals which are not volatile, may be readily extracted by known processes. The oxide of zinc rising from the ore is carried off through elbow I and pipe P, cooled by any known suitable form of condenser, and finally discharged into receivers in the form of white oxide of zinc. The sulphur contained in the ore burns in the chamber G, in cases where air is used for oxidizing, thus aiding in heating the material therein, and passes off through pipe P as sulphurous acid.

It will be seen that the process is exactly the same for the production of white oxide of

zinc, white arsenic, oxide of tellurium or oxide of antimony, the difference in product being due to the difference in the material treated.

What I claim as my invention, and desire to secure by Letters Patent, is—

The herein described method of treating ores of the class described, consisting in heating the ore in a chamber closed against the entrance of products of combustion, admitting air to the bottom of said chamber and as the process progresses gradually admitting air at points in different zones in regular succession from bottom to top, and leading off and condensing the resulting oxide, substantially as set forth.

HENRY H. EAMES.

Witnesses:

HENRY B. LOTHROP,  
AMELIA WILLIAMS.